

## UNITED STATES PATENT OFFICE

2,456,370

PROCESS FOR PRODUCING ELECTRODE-  
POSED NICKEL STRIP CONTAINING  
BORONMortimer Pierce Buck, Huntington, W. Va., as-  
signor to The International Nickel Company,  
Inc., New York, N. Y., a corporation of DelawareNo Drawing. Application April 6, 1945, Serial No.  
587,024. In Canada February 19, 1945

13 Claims. (Cl. 204--37)

1

The present invention relates to a method of introducing modifying materials into electrolytically produced metals and, more particularly, to a method for the production of electrolytic nickel suitable for rolling to blister-free nickel strip.

Heretofore, when employing electrolytically produced metal for the production of finished goods, it has been necessary to melt the electrolytically produced metal and add desirable modifying agents to the molten metal. Thus, in producing alloys of metals electrolytically produced, it has been necessary to add deoxidizers, desulfurizers, hardening agents, agents for increasing the tensile strength, agents for inducing precipitation hardening and the like to a molten charge of the electrolytically produced metal.

In many instances, even when it has not been deemed necessary or desirable to add modifying agents, the fabrication of electrolytically produced metal has been attempted with difficulty. An example of the difficulty encountered in directly utilizing electrolytically produced metal is the difficulty arising in attempting to produce nickel strip directly from nickel cathodes. The art has been confronted with the problem of producing nickel strip directly from cathode nickel without the formation of blisters on annealing. The art recognized the broad problem as early as 1921 as will be readily understood by a reference to U. S. Patent No. 1,628,149 granted to Hybinette. This patentee proposed to make malleable nickel directly from cathode nickel by rolling and annealing the cathode nickel thus produced. An important feature of Hybinette's process was the boiling of the electrolyte in such a manner that the total volume of electrolyte employed was boiled at least once every 24 hours. Later, U. S. Patent No. 2,181,936 was granted to Clappier and McDowell on a process for producing nickel strip directly from cathode nickel. The Clappier and McDowell process involved cold rolling, annealing at critical temperatures and subsequent further reduction of the annealed strip to final gauge.

It will be observed that the latter of these patented processes seek during the rolling to correct a condition existing in the metal delivered to the rolling mill which appeared to be the cause of the blisters in the finished nickel strip. It has now been discovered that blister-free nickel strip can be produced directly from cathode nickel by eliminating the source of the difficulties before the cathode nickel is introduced into the rolling mill.

It is an object of the present invention to provide cathode metal having incorporated therein

2

such modifying or addition agents as are necessary to produce the desired finished product.

It is within the purview of the present invention to provide a process for introducing modifying or addition agents such as deoxidizers, desulfurizers, hardening agents, agents for increasing tensile strength and the like into cathode metal at temperatures below the fusion point of the cathode metal.

The present invention likewise contemplates a process for producing blister-free nickel strip wherein degasifying agents are introduced into the nickel cathode before reduction in gauge.

Other objects and advantages will become apparent from the following description.

This application is a continuation-in-part of my co-pending U. S. application Serial No. 382,164, filed March 7, 1941, which has become abandoned.

Broadly speaking, the present invention involves the introduction of an elemental modifying agent into one or more portions of a metallic product, at least a part of which is composed of electrodeposited metal, followed by heat treatment to thereby cause diffusion of said modifying agent into the rest of said metallic product. The modifying agent may be introduced into the electrodeposited metal during one or more of the electrolysis steps or it may be included in a non-electrodeposited portion of the metallic product. Alternatively, the modifying agent may be applied to the surface of said metallic product in one or more stages of the preparation thereof. After introduction of the modifying agent, the metallic product is heat treated at elevated temperatures causing diffusion of the modifying agent therethrough with resultant modification of physical and chemical properties. The metallic product may be worked to desired dimensions prior to heat treatment, if necessary.

Several methods are available for introducing the modifying agent into the metallic product. Thus, for example, the modifying agent may be introduced into an electrodeposited portion of the metallic product by suspending the elemental modifying agent in the electrolyte from which a portion of the metallic product is deposited. Alternatively, a starting sheet may be supported horizontally in a plating tank and the elemental modifying agent suspended in the plating bath causing the particles of the modifying agent to settle upon the starting sheet. After electrolysis, the modifying agent is thus included between the starting sheet and the electrodeposited metal. It is also within the purview of the invention to co-

deposit the modifying agent together with the metal from the plating bath. In carrying out such a process, however, the modifying agent must be deposited in elemental form. I may also suspend a metal cathode in a molten bath containing a salt of the modifying agent in which case the atoms thereof are liberated on the surface of the cathode and go into solution in the cathode metal with resultant diffusion into the interior of the cathode due to the elevated temperature of the molten bath. On the other hand, the modifying agent may be dissolved or suspended in a molten bath from which the metal is deposited.

In another embodiment of the invention, the modifying agent may be introduced into a non-electrodeposited starting sheet. The desired amount of metal is then deposited upon the starting sheet by conventional methods. In this embodiment of the invention, the elemental modifying agent may be added to the starting sheet when the latter is in a molten condition or the starting sheet may be formed by the conventional methods of powder metallurgy from a mixture of powdered metal and modifying agent.

The modifying agent may also be applied to the surface of the metallic product during one or more stages in the formation thereof. Thus, the molten modifying agent may be applied to the surface of a starting sheet and metal plated thereon after the modifying agent has solidified. Alternatively, the vapors of the modifying agent or a suitable compound thereof, such as the hydride, may be sprayed upon the surface of the starting sheet prior to deposition. It is also within the scope of the invention to interrupt the electrodeposition at intervals and apply the molten modifying agent to the surface. Equivalently, the vapors of the modifying agent or a suitable compound thereof may be sprayed upon the surface when the deposition is interrupted.

The metallic product containing the elemental modifying agent produced by any of the methods hereinbefore discussed is then worked to desired gauge and subjected to heat treatment at elevated temperatures with resultant desired change in the physical and chemical properties thereof.

As an illustration of the principles of the present invention, the introduction of elemental boron into nickel strip may be considered. I have discovered that nickel strip containing elemental boron is substantially blister-free when exposed to temperatures in excess of about 1000° F. whereas ordinary electrolytic nickel strip is badly blistered after exposure to such a temperature.

The elemental boron may be introduced into the nickel by any of the methods referred to hereinbefore. However, I prefer to suspend powdered elemental boron in a conventional nickel plating bath from which at least a portion of the nickel strip is deposited. The amount of elemental boron to be added may vary from about 0.0001 ounce per gallon to about 0.02 ounce per gallon. The use of a greater quantity is uneconomical. Moreover, if a greater quantity is used, the elemental boron tends to interfere with the deposition of the nickel from the plating bath. On the other hand, the use of a lesser amount results in blistering of the nickel strip when exposed to temperatures above about 1000° F.

The bath is agitated during plating in order to keep the particles of elemental boron in suspension. Preferably, a stream of compressed air is blown through the bath during the deposition of the nickel, although stirring or mechanical

agitation may be utilized. I have also found it helpful to oscillate the cathode while nickel deposition is occurring. In the event that it is not desired to agitate the bath, a starting sheet may be placed horizontally in the electrolyte and the particles of metallic boron allowed to settle thereon. Nickel may then be deposited upon the starting sheet, thus entrapping the elemental boron between the starting sheet and the electrodeposited nickel.

It is to be understood that the present invention embraces the inclusion of elemental boron either in a portion of the electrodeposited metal or throughout the electrodeposited metal. Thus, 15 nickel may be plated upon a commercial nickel cathode from a conventional plating bath to which elemental boron has been added. Alternatively, nickel may be deposited upon a starting sheet from an electrolyte having elemental boron 20 suspended therein. If desired, deposition may be interrupted when not less than 0.003 inch of nickel has been plated and deposition continued in a bath free from elemental boron until a deposit of the desired thickness has been built up. 25 For best results the thickness of the cathode after electrodeposition should be from about 0.050 inch to about 0.250 inch.

After the desired thickness has been attained, the cathode is removed from the bath and annealed for the purpose of diffusing the metallic boron throughout the body of the cathode. The time and temperature of the anneal will depend on the method used to incorporate the boron in the cathode. If the boron has been deposited 30 throughout the cathode, an anneal for about 1/2 to about 2 hours at a temperature of about 1500° F. to about 2400° F. is preferred. If the boron-containing nickel plate is only a small portion of the entire cathode, then an annealing treatment 35 of about 4 to about 16 hours at a temperature of about 1500° F. to about 2400° F. is preferred. Those skilled in the art will appreciate that an annealing period of about 1/2 to about 16 hours may be utilized, the length of the period 40 depending on the thickness of the boron-containing plate as compared with the total thickness of the cathode from which the nickel strip is to be produced.

If the boron-containing plate is deposited on the surface of a boron-free cathode, some precaution must be taken to avoid the loss of boron during the anneal. The cathode may be provided with a gas-tight envelope during the annealing treatment or, alternatively, a protective atmosphere may be utilized. A protective atmosphere, in this sense, is one which is inert or non-oxidizing with respect to the modifying agent, for example elemental boron, which is used. However, if the boron has been deposited 55 throughout the cathode or if the boron-containing plate has been overlaid by a boron-free nickel plate, such precaution need not be observed.

After annealing, the cathode is hot or cold worked to produce a reduction in thickness of at 60 least 20% and preferably at least 50%. It is notable that this reduction in thickness is accomplished without edge checking or other difficulty. The nickel strip produced in accordance with the principles of the present invention has 65 a ductility of about 90 Erichsen to about 105 Erichsen, a value of 100 being taken as the average value for annealed nickel. Furthermore, the nickel strip is substantially free from blistering when exposed to temperatures in excess of 70 about 1000° F.

It is important that the boron be deposited in elemental form in order to obtain the novel results of the present invention. I am aware that a small quantity of borates is usually present in nickel deposited from conventional nickel plating baths in which boric acid is used as a buffer. However, the borates are only present in spectroscopic quantities, if at all, and the presence of borates in nickel strip does not prevent severe blistering thereof when exposed to temperatures in excess of about 1000° F. Thus, a nickel cathode plated from a conventional nickel plating bath containing approximately 30 grams per liter of boric acid, cold rolled to a thickness of about 0.020 inch and annealed at a temperature of about 2200° F. developed from about 520 to about 1730 blisters per square foot upon subsequent exposure to temperatures of excess of about 1000° F.

Cathode strip containing elemental boron and produced as herein described when exposed to temperatures appreciably in excess of 1000° F. after hot or cold working to relatively thin sections or gauge is blister-free. Relatively thin cathode nickel produced as described herein without hot or cold working, that is to say directly, when exposed to elevated temperatures in excess of 1000° F. is likewise blister-free.

A hypothesis explaining the novel results obtained by employing the process of the present invention in the production of blister-free cathode nickel strip, for example, predicates the existence of oxygen-containing occlusions in the electrodeposited metal such as water, either free or in combination, hydroxides and oxides. When such cathode metal is heated to elevated temperatures these occlusions liberate water vapor, or unite with occluded hydrogen to form water vapor. The steam pressure thus generated is sufficient to produce blisters. However, when boron is incorporated in cathode metal in accordance with the principles of the present invention, it may be predicated that the boron unites with the oxygen forming a compound which does not decompose at temperatures to which the cathode strip is subsequently exposed. Thus, the oxygen is present in a heat stable form instead of in a heat labile form and the hydrogen liberated by this reaction escapes from the cathode by diffusion.

The following illustrative examples are provided for the purpose of giving a person skilled in the art a clear understanding of the method of practicing my invention:

#### Example I

A commercial nickel cathode was suspended in a conventional Watts nickel plating bath to which about 0.014 ounce per gallon of elemental boron was added. The elemental boron was kept in suspension during the plating by agitating the bath with a stream of compressed air. Deposition of nickel was carried out at a current density of about 50 amperes per square foot, a temperature of about 140° F. and a pH of about 3.5. When the thickness of the cathode deposit reached about 0.007 inch, the cathode was removed from the bath and inserted into a gas-tight container. The cathode was then subjected to heat treatment for about 16 hours at about 2100° F. after which nickel strip was produced by cold rolling the cathode to a thickness of about 0.020 inch. Analysis of the strip disclosed an elemental boron content of about 0.001% and the nickel strip was

substantially free from blistering when exposed to temperatures higher than about 1000° F. Analysis of the cathode before electrodeposition revealed the presence of no elemental boron.

#### Example II

A passive starting sheet was suspended in a conventional nickel plating electrolyte to which about 0.014 ounce per gallon of elemental boron was added. Plating was carried out at a temperature of about 130° F., a pH of about 3.0 and a current density of about 57 amperes per square foot. The bath was agitated to insure that the metallic boron would remain in suspension. When the deposit had attained a thickness of about 0.010 inch, the cathode was removed from the electroplating bath and the boron-containing nickel plate stripped from the passive starting sheet. The sheet of boron-containing electrolytic nickel thus obtained was plated on both sides in a second nickel plating electrolyte which contained no elemental boron until a total thickness of about 0.12 inch was attained. The cathode was removed from the bath and heat treated for about 1 and 1/2 hours at a temperature of about 2250° F. The cathode was then cold rolled to a thickness of about 0.020 inch and upon analysis was found to contain about 0.005% boron. Substantial freedom from blistering was observed when said cathode nickel strip was exposed to temperatures in excess of about 1000° F.

#### Example III

A nickel starting sheet was cathodically treated in a conventional Watts bath to which about 0.0014 ounce per gallon of elemental boron was added. A temperature of about 140° F., a pH of about 3.5 and a current density of about 45 amperes per square foot were maintained during the electrolysis which was continued until a plating about 0.15 inch thick was obtained. Continuous agitation with compressed air was utilized throughout the electrodeposition to keep the elemental boron in suspension in the plating tank. The cathode was removed from the bath and subjected to diffusion for about one-half hour at a temperature of about 2100° F. The cathode was then cold rolled to a thickness of about 0.020 inch to form nickel strip which analyzed about 0.02% elemental boron. When the nickel strip was subjected to temperatures in excess of about 1000° F., substantially no blistering was observed.

The blister-free nickel strip produced as described in the preceding examples had a ductility of between about 90 Erichsen and about 105 Erichsen, a value of 100 being taken as the average value for annealed nickel.

Although the present invention has been described in conjunction with certain embodiments thereof, it is to be understood that variations and modifications may be made as those skilled in the art will readily understand. Such variations and modifications are to be considered within the purview of the specification and the scope of the appended claims. Thus, while mention has been made of boron, it is to be understood that by the term "modifying" or "addition agent" or "materials" such elements as carbon, lithium, beryllium, sodium, magnesium, aluminum, silicon, phosphorus, potassium, calcium, scandium, titanium, vanadium, chromium, manganese, rubidium, strontium, yttrium, zirconium, columbium, molybdenum, cesium, barium, lanthanum and the other rare earth elements, haf-

7  
nium, tantalum, tungsten, bismuth, thorium and uranium are also included.

Furthermore, as those skilled in the art know, the Watts bath is the conventional bath presently used for plating nickel. A typical Watts bath has the following composition and is operated under the following conditions:

|                         |             |                    |
|-------------------------|-------------|--------------------|
| Nickel sulfate          | oz./gal     | 32                 |
| Nickel chloride         | do          | 6                  |
| Boric acid              | do          | 4                  |
| pH (electrometric)      |             | 1.5-3.0 or 4.5-5.6 |
| Cathode current density | amp./sq. ft | 40                 |
| Temperature             | ° F         | 110                |

However, in practice, wide variations are made both in the composition and conditions set forth hereinbefore and I intend to include such variations by use of the term "nickel plating bath" or its derivatives in the appended claims.

I claim:

1. A process for producing electrodeposited nickel strip containing boron which comprises plating a layer of nickel having a thickness of at least 0.003 inch upon a starting sheet from an aqueous nickel plating bath containing about 0.0001 to about 0.02 ounce per gallon of powdered elemental boron, agitating the bath during plating to maintain said elemental boron suspended therein, stripping said layer of nickel from said starting sheet, plating nickel upon said layer of nickel from an electrolyte containing no elemental boron until a thickness of about 0.050 inch to about 0.250 inch is obtained, annealing the resultant cathodic electrodeposit for about ½ hour to about 2 hours at a temperature of about 1500° F. to about 2400° F., and working said cathodic electrodeposit to reduce the thickness thereof at least 20% to produce electrodeposited nickel strip having substantially no tendency to blister when exposed to temperatures in excess of about 1000° F., said electrodeposited nickel strip having a ductility of about 90 to about 105 Erichsen, a value of 100 being taken as the average value for annealed nickel.

2. A process for producing electrodeposited nickel strip containing boron which comprises plating a layer of nickel having a thickness of at least 0.003 inch upon a starting sheet from an aqueous nickel plating bath containing about 0.0001 to about 0.02 ounce per gallon of powdered elemental boron, agitating the bath during plating to maintain said elemental boron suspended therein, stripping said layer of nickel from said starting sheet, plating nickel upon said layer of nickel from an electrolyte containing no elemental boron until a thickness of at least 0.050 inch is obtained, heat treating the resultant cathodic electrodeposit for about ½ hour to about 2 hours at a temperature of about 1500° F. to about 2400° F., and working said cathodic electrodeposit to produce electrodeposited nickel strip having substantially no tendency to blister when exposed to temperatures in excess of about 1000° F.

3. A process for producing electrodeposited nickel strip containing boron which comprises electrodepositing nickel on a nickel cathode from an aqueous nickel plating bath containing about 0.0001 to about 0.02 ounce per gallon of elemental boron, agitating said plating bath to maintain the elemental boron suspended therein while oscillating said nickel cathode, removing said cathode from the electrolytic bath when a thickness of at least 0.050 inch is obtained, heat treating said nickel cathode for about ½ hour to

8  
about 2 hours at a temperature of about 1500° F. to about 2400° F., and working said nickel cathode to obtain electrodeposited nickel strip having substantially no tendency to blister when exposed to temperatures in excess of about 1000° F., said electrodeposited nickel strip containing about 0.001% to about 0.02% of elemental boron.

4. A process for producing electrodeposited nickel strip containing boron which comprises depositing nickel on a nickel cathode from an aqueous nickel plating bath containing about 0.0001 to about 0.02 ounce per gallon of elemental boron, agitating said plating bath to maintain the elemental boron suspended therein, removing said cathode from the electrolytic bath when a thickness of at least 0.050 inch is obtained, heat treating said nickel cathode for about ½ hour to about 2 hours at a temperature of about 1500° F. to about 2400° F., and working said nickel cathode to obtain electrodeposited nickel strip having substantially no tendency to blister when exposed to temperatures in excess of about 1000° F.

5. A process for producing electrodeposited nickel strip containing boron, said nickel strip having substantially no tendency to blister when exposed to temperatures in excess of about 1000° F., which comprises electroplating at least 0.007 inch of nickel upon a nickel cathode from an aqueous nickel plating bath containing about 0.0001 to about 0.02 ounce per gallon of elemental boron, passing a stream of compressed air through said plating bath while the nickel is being deposited, heat treating the resulting nickel electrodeposit for about 4 to about 16 hours at a temperature of about 1500° F. to about 2400° F., and working said nickel electrodeposit to produce nickel strip substantially free from volatile heat labile compounds of oxygen, said nickel strip having a ductility of about 90 to about 105 Erichsen, a value of 100 being taken as the average value for annealed nickel.

6. A process for producing electrodeposited nickel strip containing boron, said nickel strip having substantially no tendency to blister when exposed to temperatures in excess of about 1000° F., which comprises immersing a nickel cathode in an aqueous nickel plating bath containing about 0.0001 to about 0.02 ounce per gallon of elemental boron, electroplating at least about 0.007 inch of nickel from said plating bath, agitating the bath while the nickel is being deposited therefrom, annealing the resulting nickel electrodeposit for about 4 to about 16 hours at a temperature of about 1500° F. to about 2400° F., and rolling said nickel electrodeposit to produce nickel strip substantially free from volatile heat labile compounds of oxygen.

7. A process for introducing boron in elemental form into a nickel product, at least a portion of which is composed of electrodeposited nickel, which comprises introducing about 0.0001 to about 0.02 ounce per gallon of powdered elemental boron into an aqueous nickel plating bath from which at least a portion of said nickel product is electrodeposited at a cathode immersed therein, agitating said plating bath to maintain said boron suspended therein, heat treating said nickel product at a temperature of at least 1500° F. for at least ½ hour to thereby cause diffusion of said elemental boron throughout said nickel product, working said nickel product to desired dimensions and annealing said product at a temperature above about 1000° F.

to obtain a ductile, blister-free nickel produced without melting.

8. A process for introducing boron in elemental form into a nickel product, at least a portion of which is composed of electrodeposited nickel, which comprises suspending about 0.0001 to about 0.02 ounce per gallon of powdered elemental boron in an aqueous nickel plating bath from which at least a portion of said nickel product is electrodeposited at a cathode immersed therein, agitating said plating bath to prevent settling of said elemental boron, and heat treating said nickel product at a temperature of at least 1500° F. for at least 1/2 hour to thereby cause diffusion of said elemental boron throughout said nickel product, working said product, and annealing said product at an elevated temperature to obtain ductile, blister-free unfused nickel.

9. A process for introducing boron as a modifying agent in elemental form into a nickel product, at least a portion of which is composed of electroplated nickel, which comprises suspending about 0.0001 to about 0.02 ounce per gallon of powdered elemental boron in an aqueous nickel plating bath from which at least a portion of said nickel product is electrodeposited at a cathode immersed therein, and heat treating said nickel product at elevated temperatures to thereby cause diffusion of said elemental modifying agent throughout said nickel product, thereafter subjecting said nickel product to mechanical working and then subjecting the mechanically worked nickel product to an annealing operation to produce wrought nickel substantially devoid of blisters without resort to a melting operation.

10. A process for introducing boron as a modifying agent in elemental form into a nickel product, at least a portion of which is composed of electrodeposited nickel, which comprises introducing about 0.001% to about 0.02% of elemental boron into at least a portion of said nickel product, while electrodepositing said portion from an aqueous nickel plating bath wherein about 0.0001 to about 0.02 ounce per gallon of powdered elemental boron is suspended and annealing said nickel product at elevated temperatures to homogenize said nickel product, and thereafter subjecting said nickel product to mechanical working and to the influence of heat to produce a wrought nickel product substantially devoid of blisters without resort to a melting operation.

11. A process for producing electrodeposited nickel strip containing boron which comprises electrodepositing nickel to a thickness of at least about 0.007 inch on a section of a nickel cathode from aqueous nickel plating solution containing about 0.001 to about 0.02 ounce per gallon of elemental boron, agitating the plating bath to prevent settling of said elemental boron, oscillating said nickel cathode while the deposition proceeds, heat treating said nickel cathode for about 1/2 hour to about 16 hours at a temperature of about 1500° F. to about 2400° F. whereby the elemental boron is diffused throughout said

5 nickel cathode, and working said nickel cathode to obtain at least a 20% reduction in thickness to thereby obtain electrodeposited nickel strip having substantially no tendency to blister when exposed to temperatures in excess of about 1000° F., said nickel strip containing about 0.001% to about 0.02% of elemental boron.

10 12. A process for producing electrodeposited nickel strip containing boron which comprises depositing nickel to a thickness of at least about 0.007 inch on a portion of a nickel cathode from an aqueous nickel plating electrolyte containing about 0.0001 to about 0.02 ounce per gallon of powdered elemental boron, agitating the plating bath to prevent settling of said elemental boron, annealing said nickel cathode for about 1/2 hour to about 16 hours at a temperature of about 1500° F. to about 2400° F. to homogenize said nickel cathode, and reducing the thickness of said nickel cathode to thereby obtain electrodeposited nickel strip having substantially no tendency to blister when exposed to temperatures in excess of about 1000° F., said nickel strip having a ductility of about 90 to about 105 Erichsen, a value of 100 being taken as the average value for annealed nickel.

15 13. A process for producing electrodeposited nickel strip containing boron which comprises electroplating nickel to a thickness of at least about 0.007 inch on a portion of a nickel cathode from an aqueous nickel plating bath having about 0.0001 to about 0.02 ounce per gallon of elemental boron suspended therein, agitating said plating bath to maintain said elemental boron in suspension, heat treating said nickel cathode for about 1/2 hour to about 16 hours at a temperature of about 1500° F. to about 2400° F. whereby the elemental boron is diffused throughout said nickel cathode, and working said nickel cathode to reduce the thickness thereof whereby electrodeposited nickel strip is obtained having substantially no tendency to blister when exposed to temperatures in excess of about 1000° F.

20 25 40 45 MORTIMER PIERCE BUCK.

#### REFERENCES CITED

The following references are of record in the file of this patent:

#### UNITED STATES PATENTS

| Number    | Name             | Date          |
|-----------|------------------|---------------|
| 211,070   | Weston           | Dec. 17, 1878 |
| 850,912   | Edison           | Apr. 23, 1907 |
| 1,628,149 | Hybinette        | May 10, 1927  |
| 1,795,512 | Schmidt          | Mar. 10, 1931 |
| 2,145,745 | Armstrong et al. | Jan. 31, 1939 |
| 2,150,094 | Bieber           | Mar. 7, 1939  |
| 2,150,095 | Kayes            | Mar. 7, 1939  |
| 2,181,936 | Clappier et al.  | Dec. 5, 1939  |
| 2,236,899 | Fetz             | Apr. 1, 1941  |
| 2,289,641 | Fetz             | July 14, 1942 |

#### OTHER REFERENCES

65 Transactions of American Electrochemical Society, vol. 59 (1931), page 364.

**Certificate of Correction**

**Patent No. 2,456,370.**

**December 14, 1948.**

**MORTIMER PIERCE BUCK**

It is hereby certified that errors appear in the printed specification of the above numbered patent requiring correction as follows:

Column 3, line 71, for the word "batch" read *bath*; column 5, line 18, for "of excess" read *in excess*; column 8, line 40, for "sadi" read *said*; column 9, line 59, for "from aqueous" read *from an aqueous*;

and that the said Letters Patent should be read with these corrections therein that the same may conform to the record of the case in the Patent Office.

Signed and sealed this 24th day of May, A. D. 1949.

**[SEAL]**

**THOMAS F. MURPHY,**  
*Assistant Commissioner of Patents.*